

## UNITED STATES PATENT OFFICE.

GUSTAV GOLDMAN, OF BALTIMORE, MARYLAND.

## PROCESS OF FELTING OR MATTING FIBERS TOGETHER.

SPECIFICATION forming part of Letters Patent No. 758,244, dated April 26, 1904.

Application filed September 26, 1903. Serial No. 174,815. (No specimens.)

*To all whom it may concern:*

Be it known that I, GUSTAV GOLDMAN, a resident of Baltimore, Maryland, have invented a new and useful Improvement in Processes of 5 Felting or Matting Fibers Together, which invention is fully set forth in the following specification.

This invention relates to the art of treating fibrous materials, whether of vegetable, animal, or mineral origin or a mixture of these, 10 in such a manner that they are bound together in a felted or matted mass, preferably in sheet or similar form. In my application, Serial No. 171,288, filed on the 29th day of August, 1903, I have described and broadly 15 claimed a process of treating fibers for this purpose, which, broadly stated, consists in introducing between the fibers a binding material in a dry or finely-divided form and then 20 subsequently treating said material in such a way as to make it an active binder to the end that it may serve to bind the materials firmly 25 together, and in said application I have claimed the process broadly or generically and have also embodied therein certain specific claims directed to one particular mode of carrying out the broad inventive idea.

The present invention relates to the same art 30 of binding fibers together and is a specific embodiment of the broad invention referred to in the aforementioned application, but is not specifically claimed therein. In the aforesaid application the specific claims define a process 35 wherein the binding material is introduced between the fibers in a dry form, together with means for supplying moisture or other solvent for the binding material, whereby it is rendered capable of actively binding the fibers together.

40 The process of the present invention consists in introducing between the fibers a plurality of substances in dry form which under proper conditions will react upon each other, so as to form a different substance or composition from that originally introduced, which new substance will itself constitute a binder 45 whereby the fibers are firmly held together in a compact or matted mass.

The inventive idea involved may receive va-

rious expressions or may be exemplified by a 50 variety of forms, all of which will come within the scope of the invention. For example, there may be introduced among the fibers a plurality of substances none of which themselves would constitute a binder for the fibers, 55 but which, nevertheless, as the result of the reaction between the various ingredients are capable of forming a binder, or one or more of the plurality of substances thus introduced might be capable of being a more or less effective binding agent before the reaction due to the presence of the other substance or substances without departing from the spirit of the invention. Moreover, the substances may be introduced by sifting the same in pow- 60 dered form throughout the fluffy or lightly-separated mass of the fibers, or they may be dusted between superimposed films or layers of the fibers as the same come from a carding or similar machine.

70 One expression of the inventive idea involved which has been found to give highly satisfactory results consists in the following process, viz: Finely-divided particles of a soluble soap, as soda soap, and a salt of suitable 75 metal, as alum, are introduced between the fibers either separately or mixed together in a substantially dry state, and are subsequently treated by heat, preferably in the presence of added moisture—for example, by steam—so 80 as to cause the metal of the salt to unite with the soap and form an insoluble metallic soap which will constitute a waterproof binder for the fibers. Preferably the fibrous material is subjected to heat and pressure at 85 the time or immediately after the introduction of steam is effected, and for the purpose of effecting mechanical and continued operation and economy of production the fibers between which the substances have been intro- 90 duced, as hereinbefore indicated, are carried between heated rollers. The result of this treatment is to produce an effective binding material, which in the particular case mentioned is highly waterproof and serves to 95 bind the fibers into a felted or matted mass. In this instance the soluble soap would itself constitute a binder; but its value as a bind-

ing agent is inferior to that of the insoluble soap resulting from the chemical reaction between the soluble soap and the metallic salt. Moreover, a metallic soap not only constitutes 5 an effective binder for holding the fibers together, but it also serves to waterproof the felted or matted mass of fibers, thereby rendering the material capable of use for purposes where a non-waterproof product could 10 not be used. While soda soap and alum have been herein specified as the ingredients employed in the particular process mentioned, these substances are illustrative only, as any suitable soluble soap and metallic 15 salt could be employed for the purpose, and while the particular method of effecting the reaction consists in the treatment of these materials by steam it is not to be understood that this is the only means which could be resorted to for effecting the reaction. Any 20 substances capable of being introduced between the fibers in a dry finely-divided form and of being caused to react upon each other by proper treatment so as to form a binder 25 for the fibers and any method of treatment which will cause this reaction would be within the scope of the invention. Moreover, it is not essential for the purposes of the invention that the materials at the time they are 30 introduced between the fibers should be in the form of powder, as they might be in the form of infinitesimally thin films or finely-shredded threads or particles, it only being essential that they should be in such condition 35 that they can be readily introduced between the fibers and subsequently treated so as to bring about the desired reaction to form the binder. Moreover, the materials may be either finely distributed throughout the entire 40 mass of a single layer or sheet of the fibrous material or it may be interposed between superimposed layers thereof.

The condition herein described as a "dry" condition is meant to include any and all conditions of the material or materials which 45 will permit it or them to be introduced between the fibers in a finely-divided state, preferably as a powder or similar state of fine division. While the powdered form is preferred 50 in order that it may sift in between the fibers, this is not essential, as the materials may be, if desired, and in some instances are, finely divided into infinitesimally thin sheets or into 55 minute threads, which are introduced between films or layers of the fibers or otherwise. From the foregoing description it will be evident that for the purposes of this invention it is not essential that the materials should actually sift through the entire mass of the fibers 60 under treatment. It is equally within the invention if the materials be applied to those fibers lying near the exterior surface or surfaces of the mass of fibers under treatment or if the materials operate upon successive super-

imposed films or sheets, so as to bind the fibers 65 together into a combined felted mass.

Having thus described the invention, what is claimed is—

1. The method of treating fibers or fibrous materials which consists in introducing between the fibers a plurality of dry finely-divided materials and causing them to react so as to form a binding material whereby the fibers will be held together in a felted or matted mass. 70

2. The process of treating fibers or fibrous material which consists in introducing between the fibers a plurality of substances in dry finely-divided condition and then causing these substances to react upon each other and thus produce a new substance capable of binding 80 the fibers together. 75

3. The process of treating fibers or fibrous material which consists in introducing between the fibers a soluble soap and a salt of a metal both in powdered form, and then treating the 85 same to form an insoluble metallic soap. 85

4. The process of treating fibers or fibrous material which consists in introducing between the fibers soda soap and a salt of a metal both in dry powdered form, and then bringing 90 about the reaction between the soap and the salt to form an insoluble metallic soap. 90

5. The process of treating fibers or fibrous material which consists in introducing between the fibers a soluble soap and alum both in powdered form, and then bringing 95 about the reaction between the soap and the alum to form an aluminium soap. 95

6. The process of treating fibers or fibrous material which consists in introducing between the fibers a plurality of substances and then subjecting the same to heat whereby said substances are caused to react and form a new substance constituting a binder for the fibrous material. 100 105

7. The process of treating fibers or fibrous material which consists in introducing between the fibers a plurality of substances in powdered form capable of reacting upon each other to produce a new substance and then subjecting said substances to heat and pressure whereby a binding substance is formed and the fibers are effectively bound together. 110

8. The process of treating fibers or fibrous material which consists in introducing between the fibers a plurality of substances in powdered form capable of reacting so as to form a binding substance, and then subjecting said substances to heat and pressure in the presence of moisture whereby a binding substance 115 120 is formed and the fibers are bound together. 120

9. The process of treating fibers and fibrous material which consists in introducing between the fibers a soluble soap and a salt of a metal both in powdered form, and then subjecting 125 the same to heat whereby an insoluble metallic soap is formed which serves to bind the fibers together. 125

10. The process of treating fibers or fibrous material which consists in introducing between the fibers a soluble soap and a salt of a metal both in powdered form, and then subjecting the same to heat and pressure whereby an insoluble waterproof soap is formed which serves to bind the fibers together.

11. The process of treating fibers or fibrous material which consists in introducing between the fibers a soluble soap and a salt of a metal both in powdered form, and then subjecting the same to heat and pressure whereby an insoluble waterproof metallic soap is formed which serves to bind the fibers together in a felted mass.

12. The process of treating fibers or fibrous material which consists in introducing between the fibers a soda soap and a salt of a metal both in powdered form, and then subjecting the same to heat and pressure in the presence of moisture whereby an insoluble metallic soap is formed which serves to bind the fibers together.

13. The process of treating fibers or fibrous material which consists in introducing between the fibers a soluble soap and alum both in powdered form, and then bringing about a reaction between the soap and the alum in the presence of heat and pressure whereby a metallic soap is formed which serves to bind the fibers together in a felted mass.

14. The process of treating fibers or fibrous material which consists in introducing between the fibers a soda soap and a salt of a metal both in powdered form and then bringing about the reaction between the soap and the salt in the presence of heat and pressure whereby a metallic waterproof soap is formed which serves to bind the fibers together in a felted mass.

15. The process of treating fibers or fibrous material which consists in introducing between the fibers soda soap and alum both in powdered form, and then bringing about the reaction between the soap and the alum in the presence of heat and pressure whereby an aluminium soap is formed which serves to bind the fibers together in a felted mass.

16. The process of treating fibers or fibrous

materials which consists in introducing between the fibers a plurality of substances and then causing said substances to react and form a new substance constituting a binder for the fibrous materials by subjecting said substances to the action of steam.

17. The process of treating fibers or fibrous materials which consists in introducing between the fibers a plurality of substances and then causing said substances to react and form a new substance constituting a binder for the fibrous materials by subjecting said substances to the action of steam and pressure.

18. The process of treating fibers or fibrous material which consists in introducing between the fibers a soluble soap and the salt of a metal both in powdered form, and then subjecting the same to the action of steam whereby an insoluble metallic soap is formed that serves to bind the fibers together.

19. The process of treating fibers or fibrous material which consists in introducing between the fibers a soluble soap and the salt of a metal, both in powdered form, and then subjecting the same to the action of steam and pressure, whereby an insoluble metallic soap is formed that serves to bind the fibers together.

20. The process of treating fibers or fibrous material which consists in introducing between the fibers a soluble soap and alum both in powdered form, and then subjecting the same to the action of steam, whereby an aluminium soap is formed which serves to bind the fibers together in a felted mass.

21. The process of treating fibers or fibrous material which consists in introducing between the fibers a soluble soap and alum both in powdered form, and then subjecting the same to the action of steam and pressure, whereby an aluminium soap is formed which serves to bind the fibers together in a felted mass.

In testimony whereof I have signed this specification in the presence of two subscribing witnesses.

GUSTAV GOLDMAN.

Witnesses:

ARTHUR LEE BROWNE,  
FRANCIS T. HOMER.